

# UNITED STATES PATENT OFFICE.

ROBERT PHILIP, OF BOFORS, SWEDEN.

## CANDLESTOCK.

1,229,132.

Specification of Letters Patent.

Patented June 5, 1917.

No Drawing.

Application filed July 29, 1916. Serial No. 112,192.

*To all whom it may concern:*

Be it known that I, ROBERT PHILIP, a subject of the King of Sweden, residing at Bofors, in the county of Örebro and Kingdom of Sweden, have invented new and useful Improvements in Candlestock, of which the following is a specification.

This invention relates to a novel material for producing candles and has for its object 10 to provide a candle, the body of which is substantially white in color, at least as white as a stearin candle. Another object is to provide a candle with a body strong enough to resist the high temperatures in 15 the torrid zones without danger of softening.

Pure paraffin candles are rarely manufactured but the so-called "paraffin candles" are often made of a mixture of paraffin with 20 some stearin, which latter is added for the purpose of facilitating the removal of the candles from the molds. Candles with a stearin content of about 15% to 50% are usually called "composition candles" and 25 show the characters mentioned.

It has been proposed to harden paraffin candles by molding a mixture of paraffin and stearin by which addition the otherwise transparent paraffin candles become 30 more opaque, of a white color and harder, than candles made of paraffin alone. A too high percentage of stearin will, however, lower the melting point in an undue degree. For instance, a percentage of 25% 35 stearin effects a lowering in the melting point of a pure paraffin candle mass by about 2 to 3 degrees centigrade, and 50% stearin lowers the melting point as much as 10 degrees centigrade, owing to the formation 40 of a so-called "eutectic" or easily fusible mixture.

Also other substances which dissolve in molten paraffin will cause the same effect. For this reason it is desirable that only a 45 small quantity of the hardening material be added. The hardening substances hitherto used, are mostly substances the melting point of which lies considerably above the melting point of paraffin, for instance soaps 50 of fatty acids (as stearate or palmitate of ammonium) amids or anilids of fatty acids, waxes, as carnauba wax or similar substances.

For technical and economical reasons, however, these last mentioned materials 55 have not been extensively used.

This invention resides in the use of materials, of which a small quantity is capable of exercising an advantageous influence on the character of the candle mass. Experience has proved that salicylic acid is a very suitable substance for this purpose. Even an addition of about  $\frac{1}{2}$  to 1% of said substance to the candle mass produces a considerable alteration in the characters of 60 the mass. The transparency decreases, so that a candle produced of this mixture looks white, and with a somewhat increased percentage of salicylic acid, 65 candles whiter than those made of stearin 70 are produced, the flexibility of the candle decreases and the fractured surfaces are finely grained. The hardness increases with the percentage of salicylic acid used.

The reason for the changes in the physical properties of the candles, by the addition of salicylic acid appears to be that the salicylic acid is originally dissolved in the fused paraffin, and upon cooling the acid 75 is separated out as very small crystals, 80 which in turn cause the paraffin to also assume a finely granular condition, during the hardening. This produces a very fine net work, which can be considered as a supporting frame, thereby producing the decreased flexibility, also to a certain extent, 85 the increased hardness. The solidification temperature is lowered by the addition of the small amounts of salicylic acid referred to above, by about 1° centigrade. 90

In making candles it is preferable to add a small percentage of stearin or similar material, for making the candles readily removable from the molds, also for making the candles more fusible. The fusibility of 95 mixtures of stearin and paraffin is more favorable than with pure paraffin, and also the addition of stearin facilitates the fine distribution in the mass of salicylic acid employed.

In the production of the candle mixture, the salicylic acid may be dissolved in the melted stearin and added to the melted paraffin, or the salicylic acid may be dissolved in the melted mixture of stearin and 105 paraffin.

Without limiting myself to specific proportions, I give the following examples of mixtures suitable for use in making candles.

|                | A   | B   |
|----------------|-----|-----|
| Paraffin       | 79% | 88% |
| Stearin        | 20% | 10% |
| Salicylic acid | 10% | 2%  |

10. For making candles for ordinary purposes, I prefer generally to employ about 10% of the stearin, although I do not desire to limit myself to this proportion.

Copies of this patent may be obtained for five cents each, by addressing the "Commissioner of Patents, Washington, D. C."

What I claim is:

1. The herein described material for making candles which contains paraffin and salicylic acid. 15

2. The herein described material for making candles which comprises paraffin, stearin and salicylic acid. 20

In testimony whereof I have affixed my signature in presence of two witnesses.

ROBERT PHILIP.

Witnesses:

GUSTAF SETH,  
ADOLF MÖLIN.